

[54] METHOD FOR PRODUCING GRAIN ORIENTED SILICON STEEL COMPRISING COPPER

[75] Inventors: James A. Salsgiver; Gerald L. Houze, Jr.; Stuart L. Ames, all of Sarver, Pa.

[73] Assignee: Allegheny Ludlum Industries, Inc., Pittsburgh, Pa.

[22] Filed: May 7, 1973

[21] Appl. No.: 357,969

**Related U.S. Application Data**

[63] Continuation-in-part of Ser. No. 293,194, Sept. 28, 1972, abandoned.

[52] U.S. Cl. .... 148/112, 75/123 L, 148/31.55, 148/111

[51] Int. Cl. .... H01f 1/04

[58] Field of Search ..... 148/111, 110, 112, 31.55; 75/123 L

[56] **References Cited**

UNITED STATES PATENTS

|           |         |                     |         |
|-----------|---------|---------------------|---------|
| 2,867,558 | 1/1959  | May et al. ....     | 148/111 |
| 3,159,511 | 12/1964 | Tagucai et al. .... | 148/111 |
| 3,266,955 | 8/1966  | Taguchi et al. .... | 148/111 |
| 3,287,183 | 11/1966 | Taguchi et al. .... | 148/111 |
| 3,700,506 | 10/1972 | Tanaka et al. ....  | 148/111 |
| 3,575,739 | 4/1971  | Fiedler.....        | 148/111 |

|           |         |                      |         |
|-----------|---------|----------------------|---------|
| 3,632,456 | 1/1972  | Sakakura et al. .... | 148/111 |
| 3,671,337 | 6/1972  | Kumai et al. ....    | 148/111 |
| 3,764,406 | 10/1973 | Littmann .....       | 148/111 |
| 3,770,517 | 11/1973 | Gray et al. ....     | 148/111 |

**OTHER PUBLICATIONS**

Kussmann, A. et al; Gekupferter Stahl For Dynamo-Und Transformatoren Bleche, in Stahl & Eisen, 50, 1930, pp. 1194-1197.

*Primary Examiner*—Walter R. Satterfield

*Attorney, Agent, or Firm*—Vincent G. Gioia; Robert F. Dropkin

[57] **ABSTRACT**

Silicon steel alloy melt composition and method for forming grain oriented silicon steel sheets therefrom, characterized in that the resulting sheets have a cube-on-edge texture with permeabilities at 10 oersteds as high as or higher than 1850. The alloy from which the steel is formed preferably contains silicon, sulfur, aluminum, manganese, nitrogen and copper. Maximum permeability is obtained when the steel being processed has a ratio (by weight) of manganese equivalent to sulfur of greater than 2.0 and less than 4.75. It is essential to provide both nitride and sulfide formers which act as primary grain growth inhibitors in a duplex primary grain growth inhibition system to effect the desirable results of the invention.

**5 Claims, 2 Drawing Figures**

PATENTED DEC 17 1974

3,855,018



## METHOD FOR PRODUCING GRAIN ORIENTED SILICON STEEL COMPRISING COPPER

This application is a continuation-in-part of now abandoned copending application Ser. No. 293,194 filed Sept. 28, 1972.

### BACKGROUND OF THE INVENTION

Oriented silicon steel sheets produced in accordance with known techniques typically have permeabilities of 10 oersteds of about 1790 to 1840, 60 Hz. core losses of about 0.490 to 0.530 watts per pound at 15 KG, and core losses of about 0.700 to 0.800 watts per pound at 17 KG for 0.011 inch gage material. Oriented silicon steels of this type, in addition to containing about 3.2 percent silicon, also contain residual elements.

In U.S. Pat. No. 3,287,183 issued to Taguchi et al, there is disclosed a process for producing a single-oriented silicon steel having a permeability of up to 1910 at 10 oersteds. The steel disclosed in the aforesaid U.S. Pat. No. 3,287,183 is processed with a light-heavy cold reduction sequence incorporating a high temperature intermediate anneal. The patent indicates that the primary recrystallization inhibitor is aluminum nitride, and that precise control defined mathematically, must be maintained over the aluminum-sulfur ratio. The best of the product described in the aforesaid patent has a much better cube-on-edge texture and higher permeability than most prior art single oriented silicon steels. In a more recently issued U.S. Pat. No. 3,636,579, there is disclosed the production of high quality material by optimizing the aluminum nitride precipitation by utilization of quenching in the process.

### SUMMARY OF THE INVENTION

In accordance with the present invention, silicon steel is provided containing critical amounts of "manganese equivalent" and sulfur, with the weight ratio of "manganese equivalent" to sulfur being in the range of 2.0 to 4.75, preferably 2.5 to 4, and having permeabilities at 10 oersteds as high as or higher than 1850 and capable of achieving permeabilities of 1940 to 1950. This steel is processed either by conventional practices or the modified practice of this invention, to produce oriented silicon steel product. The term "manganese equivalent" as used herein means the weight percent manganese plus  $n$  times the weight percent copper, where  $n$  is a number in the range 0.1 to 0.25. Allowance must be made for the presence of copper because, like manganese it is a sulfide former and will affect sulfide formation. In contrast to the teachings of the aforesaid U.S. Pat. No. 3,287,183, which prescribes criticality of the aluminum to sulfur ratio to achieve high permeabilities, it has been found that high permeabilities are achieved by controlling the ratio of manganese equivalent to sulfur and the amount of aluminum nitride component.

Further, it has been found that it is preferred to utilize a hot rolled band anneal, 10 seconds to 30 minutes, preferably 10 seconds to 5 minutes, at a temperature of at least 1400°F to produce, more consistently, the desired high permeability at 10 oersteds of 1850 or higher.

### DESCRIPTION OF THE PREFERRED EMBODIMENTS

The above and other objects and features of the invention will become apparent from the following de-

tailed description taken in connection with the accompanying drawings which form a part of this specification, and in which:

FIG. 1 is a plot of manganese equivalent-sulfur ratio versus permeability for various steels processed in accordance with the teachings of the invention; and

FIG. 2 is a plot of core loss versus permeability for steels processed in accordance with the teachings of the invention.

The steels of the invention can be melted to the following ranges of composition and processed to final product:

|                                                     |                           |        |
|-----------------------------------------------------|---------------------------|--------|
| Carbon                                              | .02                       | -.07%  |
| Manganese equivalent<br>(%Mn + (0.1 to 0.25) × %Cu) | .05                       | -.24%  |
| Sulfur                                              | .01                       | -.05%  |
| Silicon                                             | 2.5                       | -.3.5% |
| Aluminum                                            | .015                      | -.04%  |
| Nitrogen                                            | 30 - 90 parts per million |        |
| Copper                                              | up to 0.3%                |        |
| Iron                                                | Balance                   |        |

and other normal steel making residuals, and wherein the ratio of manganese equivalent to sulfur, by weight, is in the range of 2.0 to 4.75, preferably 2.5 to 4. It is also desirable to have at least 0.1 percent copper present as copper is believed to lower annealing temperatures, improve rollability and relax annealing atmosphere requirements.

Conventional processing to produce oriented silicon steel product generally includes:

1. preparing a melt of steel and casting same into ingots,
2. hot rolling ingot to hot rolled band,
3. cold rolling the hot rolled band,
4. annealing the cold rolled steel,
5. cold rolling again,
6. decarburize annealing,
7. coating (optional) with suitable separator, e.g. MgO slurry, and
8. final texture (desulfurize) annealing.

As was mentioned above, the improved processing of the steel of the invention involves certain critical steps. In particular, the processing in accordance with the invention includes hot rolled band heat treatment to a temperature above 1400°F, (e.g. 1400°F-2100°F) preferably 1650-1850°F, for 10 seconds to 30 minutes, preferably 10 seconds to 5 minutes, prior to subsequent processing.

In order to illustrate the effects of the invention, twelve vacuum induction melted heats were made. The melt characteristics are shown in the following Table I for these twelve heats:

TABLE I

| Heat*     | Mn   | S    | Si   | Cu   | Al   | N<br>ppm |
|-----------|------|------|------|------|------|----------|
| RV-3822A  | .13  | .026 | 2.75 | .085 | .009 | 24       |
| RV-3822B  | .13  | .033 | 2.75 | .085 | .014 | 31       |
| RV-3822C  | .13  | .042 | 2.75 | .085 | .022 | 41       |
| RV-3823A  | .13  | .025 | 2.77 | .086 | .016 | 58       |
| RV-3823B  | .13  | .033 | 2.77 | .086 | .020 | 66       |
| RV-3823C  | .13  | .044 | 2.77 | .086 | .029 | 83       |
| RV-3831   | .062 | .020 | 2.82 | .012 | .007 | 31       |
| RV-3856   | .12  | .026 | 2.72 | .082 | .020 | 60       |
| RV-3857   | .12  | .029 | 2.83 | .085 | .026 | 65       |
| RV-3858   | .048 | .038 | 2.70 | .075 | .030 | 68       |
| RV-4970   | .12  | .044 | 2.73 | .10  | .016 | 56       |
| RV-5370** | .054 | .023 | 2.80 | .31  | .025 | 68       |

\*Other elements present in typical residual amounts, e.g. carbon 0.02 to 0.07%, nickel 0.02% to 0.043%, chromium 0.01 to 0.018.

\*\*Heat RV-5370 was divided into ingots RV-5370 and RV-5370(S).

Included in Table I is a control heat (RV-3831) with a conventional oriented composition except for the somewhat low silicon content. The ingots were hot rolled to a band thickness of about 125 mils, except for RV-5370(S) which was rolled to 90 mils, after a 1-hour soak at 2500°F. Hot rolled band samples from each heat were given the following heat treatments:

1. No hot rolled band heat treatment.
2. Two minutes at 1650°F.
3. Thirty minutes at 1830°F. After the hot rolled band treatment, all the band samples were surface conditioned and rolled to an intermediate gage of 84 mils, (except for RV-5370(S) which was already at 90 mils) a reduction of about 33 percent. Each sample, including RV-5370(S) was then halved, and two choices of heat treatment were used as a high temperature normalize. The first normalize consisted of a heat treatment of five minutes above 1875°F (with a maximum temperature of about 1905°F) in a protective atmosphere (hydrogen-nitrogen mixture). The other normalize was an anneal for five minutes above 1960°F with a maximum temperature of 2010°F, also in a protective atmosphere.

After the normalize, all materials were cold rolled to nominally 11 mils, a reduction of approximately 87 percent, and final normalized for 1 minute at 1475°F in a decarburizing atmosphere. Samples, measuring 15.25 cm x 3 cm were sheared for final annealing and used for evaluation of electrical properties.

The final annealing practice consisted of heating to 2150°F. Hydrogen was used to purify the steel and sulfur was removed at this stage of the processing. In the conventional production of oriented silicon steel it is desirable to remove all impurities possible at or near the final stages of the process. Thus, for example, the final chemistry will be low in carbon, sulfur and aluminum. The removal of the latter preferably occurs by oxidation and absorption into surface coatings such as MgO.

The effects of composition, hot rolled band treatment and intermediate normalizing on the texture as condensed into the following Table II.

TABLE II

| Heat       | Permeability at 10H as a Function of Heat Treatment at Various Stages of Processing |        |                   |                                           |                      |
|------------|-------------------------------------------------------------------------------------|--------|-------------------|-------------------------------------------|----------------------|
|            | High Temperature Norm.<br>1900°F                                                    | 2000°F | No Heat Treatment | HRB Heat Treatment<br>2 Min.<br>at 1650°F | 30 Min.<br>at 1850°F |
| RV-3822A   | X                                                                                   |        | 1405              | 1410                                      | 1513                 |
| RV-3822A   |                                                                                     | X      | 1423              | 1414                                      | 1617                 |
| RV-3822B   | X                                                                                   |        | 1432              | 1472                                      | 1477                 |
| RV-3822B   |                                                                                     | X      | 1439              | 1449                                      | 1549                 |
| RV-3822C   | X                                                                                   |        | 1749              | 1852                                      | 1848                 |
| RV-3822C   |                                                                                     | X      | 1594              | 1941                                      | 1667                 |
| RV-3823A   | X                                                                                   |        | 1670              | 1759                                      | 1641                 |
| RV-3823A   |                                                                                     | X      | 1441              | 1439                                      | 1455                 |
| RV-3823B   | X                                                                                   |        | 1747              | 1863                                      | 1823                 |
| RV-3823B   |                                                                                     | X      | 1780              | 1880                                      | 1881                 |
| RV-3823C   | X                                                                                   |        | 1810              | 1830                                      | 1821                 |
| RV-3823C   |                                                                                     | X      | 1815              | 1915                                      | 1831                 |
| RV-3831    | X                                                                                   |        | 1382              | 1389                                      | 1426                 |
| RV-3831    |                                                                                     | X      | 1389              | 1391                                      | 1427                 |
| RV-3856    | X                                                                                   |        | 1706              | lost                                      | 1831                 |
| RV-3856    |                                                                                     | X      | 1723              | lost*                                     | 1863                 |
| RV-3857    | X                                                                                   |        | 1815              | 1844                                      | 1809                 |
| RV-3857    |                                                                                     | X      | 1809              | 1907                                      | 1830                 |
| RV-3858    | X                                                                                   |        | 1639              | 1668                                      | 1662                 |
| RV-3858    |                                                                                     | X      | 1571              | 1500                                      | 1528                 |
| RV-4970    |                                                                                     | X      |                   | 1910                                      |                      |
| RV-5370(S) | none                                                                                | X      |                   | 1910**                                    |                      |
| RV-5370    |                                                                                     | X      | 1897              |                                           |                      |

\*Single strip samples lost; however, later a pack sample was generated for this condition and it had a  $\mu$  at 10H = 1901.

\*\*2 min. at 1830°F.

A study of Table II indicates that the best heats were RV-3822C, RV-3823B, RV-3823C, RV-3857 and RV-5370. Table II shows that to develop the highest permeabilities for the examples given, it is desirable to have a hot rolled bond heat treatment as described. As regards the intermediate anneal, note that heats RV-3823B and RV-3823C which were annealed at 1900°F have lower permeability values than those subjected to the 2000°F anneal. The permeability values listed in Table II are the result of single strip tests with the one exception noted.

It has been determined that in almost all cases, the hot band heat treatment of about 1400°F produces the best permeability. Table II illustrates this effect.

The effects of manganese equivalent on final permeability are shown in FIG. 1, wherein the permeability is plotted as a function of the manganese equivalent-sulfur ratio for a set of samples from Table II processed under conditions giving high permeability values. It is apparent that the manganese equivalent-sulfur ratio is optimized at around 3. The poor permeability heats (RV-3831, RV-3822B and RV-3822A) are those with low aluminum content ranging from .007 to 0.014 percent. The heats with values on the curve have aluminum contents ranging from 0.016 to 0.030. This demonstrates the synergistic effect of both sulphides and nitrides as primary grain growth inhibitors in these materials.

The core losses decrease as permeability increases as shown in FIG. 2 wherein the 17KG values are confined generally between lines 10 and 12 while the 15 KG values are confined between lines 14 and 16. Thus, an increase in permeability also results in an enhancement of core loss characteristics.

Although the invention has been shown in connection with certain specific embodiments, it will be readily apparent to those skilled in the art that various changes in composition and process steps can be made to suit requirements without departing from the spirit and scope of the invention.

We claim:

1. In a process for producing oriented silicon steel including the step of preparing a melt of steel and casting

same into ingots, hot rolling said ingots to hot rolled band gauge and subsequently cold rolling and annealing, as desired to produce silicon steel with cube-on-edge orientation, the improvement which comprises preparing a melt of steel having a composition consisting essentially of:

|                                                     |                           |   |      |
|-----------------------------------------------------|---------------------------|---|------|
| Carbon                                              | .02                       | – | .07% |
| Manganese equivalent<br>(%Mn + (0.1 to 0.25) × %Cu) | .05                       | – | .24% |
| Sulfur                                              | .01                       | – | .05% |
| Silicon                                             | 2.5                       | – | 3.5% |
| Aluminum                                            | .015                      | – | .04% |
| Nitrogen                                            | 30 – 90 parts per million |   |      |
| Copper                                              | 0.1 to 0.3%               |   |      |
| Iron                                                | Balance                   |   |      |

and wherein the ratio of manganese equivalent to sulfur, by weight, is in the range of 2.0 to 4.75, and thereafter processing said steel to produce grain oriented steel with cube-on-edge texture whereby said oriented

steel has a permeability of at least 1850 at 10 oersteds due to a duplex sulfide and nitride primary grain growth inhibition system, said system resulting from the aforementioned chemistry of the steel processed; said processing including the step of subjecting said hot rolled band to a temperature above 1400°F for 10 seconds to 30 minutes, said hot rolled band heat treatment contributing to the attainment of said high permeability for said oriented silicon steel.

5 10 2. An improvement according to claim 1, wherein the ratio of manganese equivalent to sulfur is 2.5 to 4.

3. An improvement according to claim 1 wherein said hot rolled band is heated to 1400°F to 2100°F.

4. An improvement according to claim 1 wherein said hot rolled band is heated to 1650°F to 1850°F.

5. An improvement according to claim 4 wherein said hot rolled band is heated to 1650°F to 1850°F for 10 seconds to 5 minutes.

\* \* \* \* \*

20

25

30

35

40

45

50

55

60

65



US003855018A

## REEXAMINATION CERTIFICATE (2190th)

United States Patent [19]

Salsgiver et al.

[11] B1 3,855,018

[45] Certificate Issued Jan. 18, 1994

[54] METHOD FOR PRODUCING GRAIN  
ORIENTED SILICON STEEL COMPRISING  
COPPER[75] Inventors: James A. Salsgiver; Gerald L. Houze,  
Jr.; Stuart L. Ames, all of Sarver, Pa.[73] Assignee: Allegheny Ludlum Corp., Pittsburgh,  
Pa.

## Reexamination Requests:

No. 90/002,300, Mar. 19, 1991

No. 90/002,013, Apr. 27, 1990

## Reexamination Certificate for:

Patent No.: 3,855,018

Issued: Dec. 17, 1974

Appl. No.: 357,969

Filed: May 7, 1973

## Related U.S. Application Data

[63] Continuation-in-part of Ser. No. 293,194, Sep. 28, 1972,  
abandoned.[51] Int. Cl.<sup>5</sup> ..... H01F 1/04[52] U.S. Cl. ..... 148/112; 148/111;  
148/308

[58] Field of Search ..... 148/111, 112, 113, 308

## [56] References Cited

## U.S. PATENT DOCUMENTS

|           |         |                 |         |
|-----------|---------|-----------------|---------|
| 2,534,141 | 12/1950 | Morrill et al.  | 148/111 |
| 2,867,557 | 1/1959  | Crede et al.    | 148/111 |
| 2,913,361 | 11/1959 | Fitz            | 148/111 |
| 3,144,363 | 8/1964  | Aspden et al.   | 148/111 |
| 3,438,820 | 4/1969  | Goss et al.     | 148/110 |
| 3,632,456 | 1/1972  | Sakakura et al. | 148/111 |
| 3,636,579 | 1/1972  | Sakakura et al. | 148/111 |
| 3,671,337 | 6/1972  | Kumai et al.    | 148/111 |
| 3,873,380 | 3/1975  | Malagari        | 148/111 |
| 3,873,381 | 3/1975  | Jackson         | 148/111 |

## FOREIGN PATENT DOCUMENTS

4710 6/1958 Japan ..... 148/111

## OTHER PUBLICATIONS

Graham, C. D., *Magnetism and Metallurgy*, ch. XV, pp. 723-742, Academic Press (1969).Leslie, William C., *The Physical Metallurgy of Steels*, 1981, p. 320.Bozarth, R., *Ferromagnetism*, 1951, p. 75.  
Iwayama K., Kuroki K., Yoshitomi Y., "Roles of Tin and Copper in the .23mm High Permeability Grain Oriented Silicon Steel", *Journal of Applied Physics*, March 15, 1984, pp. 2136-2138.Shen, T. H., "The Study of Second Phase Particles in Grain Oriented 3% Si-Fe" *Journal of Materials Engineering*, Vol. 11, No. 1, 1989, pp. 71-82.Nakashima, Takashima & Harase, "Effect of Silicon Content on Secondary Recrystallization . . .", *ISIJ International*, Vol. 31, 1991, pp. 1007-1012.Nakashima, Takashima & Harase, "Effect of Cold Rolling Reduction on Secondary Recrystallization . . .", *ISIJ International*, Vol. 31, 1991, pp. 1013-1019.Kiessling, Westman C., "Sulphide Inclusions and Synthetic Sulphides of the (Mn,Me)S Type", *Jnl. Iron & Steel Institute*, 1986, pp. 377-379.

Primary Examiner—George Wyszomierski

[57] ABSTRACT  
Silicon steel alloy melt composition and method for forming grain oriented silicon steel sheets therefrom, characterized in that the resulting sheets have a cube-on-edge texture with permeabilities at 10 oersteds as high as or higher than 1850. The alloy from which the steel is formed preferably contains silicon, sulfur, aluminum, manganese, nitrogen and copper. Maximum permeability is obtained when the steel being processed has a ratio (by weight) of manganese equivalent to sulfur of greater than 2.0 and less than 4.75. It is essential to provide both nitride and sulfide formers which act as primary grain growth inhibitors in a duplex primary grain growth inhibition system to effect the desirable results of the invention.

**REEXAMINATION CERTIFICATE  
ISSUED UNDER 35 U.S.C. 307****NO AMENDMENTS HAVE BEEN MADE TO  
THE PATENT****AS A RESULT OF REEXAMINATION, IT HAS  
BEEN DETERMINED THAT:**

5 The patentability of claims 1-5 is confirmed.

\* \* \* \* \*

10

15

20

25

30

35

40

45

50

55

60

65